

March 2, 1937.

H. K. MOORE

2,072,177

MANUFACTURE AND REFINEMENT OF CHEMICAL PULPS AND  
REGENERATION OF THE SPENT CHEMICAL LIQUORS

Filed Oct. 24, 1933

3 Sheets-Sheet 1



Inventor  
Hugh K. Moore  
By Wright, Brown, Simby, May  
Attest

March 2, 1937.

H. K. MOORE

2,072,177

MANUFACTURE AND REFINEMENT OF CHEMICAL PULPS AND  
REGENERATION OF THE SPENT CHEMICAL LIQUORS

Filed Oct. 24, 1933

3 Sheets-Sheet 2



*W. K. Moore*  
Inventor  
Hugh K. Moore  
3 Wright, Bronx, New York  
*W. K. Moore*

March 2, 1937.

H. K. MOORE

2,072,177

MANUFACTURE AND REFINEMENT OF CHEMICAL PULPS AND  
REGENERATION OF THE SPENT CHEMICAL LIQUORS

Filed Oct. 24, 1933

3 Sheets-Sheet 3



Inventor  
Hugh K. Moore  
7 Wright, Brown, Quincy, Mass.

Attn:

## UNITED STATES PATENT OFFICE

2,072,177

MANUFACTURE AND REFINEMENT OF  
CHEMICAL PULPS AND REGENERATION  
OF THE SPENT CHEMICAL LIQUORSHugh K. Moore, Berlin, N. H., assignor to Brown  
Company, Berlin, N. H., a corporation of  
Maine

Application October 24, 1933, Serial No. 694,996

18 Claims. (Cl. 23—46)

This invention relates to the manufacture and refinement of chemical pulps, including the regeneration of spent chemical liquors such as are available in the pulp-making and pulp-refining industries, and deals more particularly to novel steps for controlling the composition of the regenerated liquors so that they may be used and regenerated most advantageously in the manufacture of pulp from wood or other raw cellulosic materials and/or in the refinement of cellulose pulps. While the principles of my invention are applicable to various kinds of spent liquors of the foregoing class which are subjected to a regenerating process involving the smelting of the inorganic compounds of the spent liquors and the causticization of the smelted inorganic compounds, nevertheless, they have particular utility and advantage in the regeneration of spent so-called kraft cooking liquors and spent liquors resulting from the step of refining preliberated cellulose pulps of the nature of kraft, sulphite, or the like, with refining liquors of a composition similar to that of the usual kraft cooking liquors, according to which causticization is performed on smelted compounds containing sodium carbonate and sodium sulphate as main constituents.

In the production of kraft pulp, it is the practice to cook the raw wood chips in an alkaline liquor whose active or fiber-liberating constituents are essentially caustic soda and sodium sulphide. Strictly speaking, the sodium sulphide does not act as such in the cooking liquor but hydrolyzes in water to furnish caustic soda and sodium hydrosulphide as the active agents of the cooking liquor, so that the cooking liquor is really richer in caustic soda than the formula showing the presence of sodium sulphide therein would indicate. The sodium hydrosulphide is not active in the same sense as is the caustic soda, notwithstanding generally held opinion to the contrary. The fact is that the sodium hydrosulphide does not split up the lignocelluloses into cellulose fiber and lignin to any appreciable extent, but it does influence the way in which the lignocelluloses are split up by the caustic soda in that it is a powerful reducing agent and inhibits the formation of oxycelluloses or other oxycellulose compounds from the cellulose fiber as it is being liberated. The sodium hydrosulphide is hence an active agent in the cooking liquor, but its function and activity is quite different from that of the caustic soda. Nevertheless, for the purpose of convenience, I shall hereinafter speak about the active constituents of a

kraft cooking liquor as consisting of caustic soda and sodium sulphide or sodium hydrosulphide. After a batch of raw wood chips have been reduced to pulp in a kraft cooking liquor, it is the practice to blow the digester in which the cooking was effected and then to separate or wash the spent cooking liquor from the raw kraft pulp in suitable washing equipment. The separated spent cooking liquor is partly returned to the digesters and partly regenerated in the form of a solution of a mixture of fresh caustic soda and sodium sulphide which is admixed with the spent cooking liquor in the production of the kraft pulp.

In regenerating the spent cooking liquor, various processes have been followed, all of which are designed, however, to yield a solution containing a mixture of caustic soda and sodium sulphide. One well known regenerating process, which is disclosed in my Patent No. 1,137,780, dated May 4, 1915, involves concentrating the spent or black liquor to a solids content, including both organic and inorganic solids, of about 50%, at which content the liquor is heated in a confined system to a high internal pressure and is then exploded as a spray directly into a furnace for the purpose of effecting a combustion of the organic content of the liquor and a smelting of its inorganic content into a molten mass of inorganic compounds containing essentially sodium carbonate and sodium sulphide as the furnace effluent. Inasmuch as losses of sodium and sulphur constituents in the cycle must be made up, this is done by adding sodium sulphate (salt cake) to the concentrated black liquor before heating it under pressure. The molten or smelted inorganic compounds coming from the furnace are discharged into a body of water to form a hot solution which contains sodium carbonate, sodium sulphide, residual sodium sulphate, and smaller amounts of sodium thiosulphate, sodium sulphite, and sodium silicate. The hot solution thus formed is delivered to a causticizing tank and lime is added thereto so as to convert the sodium carbonate into caustic soda. The resulting causticized solution is then allowed to stand to ensure a settling of the precipitated calcium carbonate and other solids, is decanted, and then delivered to a storage tank from which liquor is withdrawn as needed for the digesters. To the storage tank liquor is added the first washings of the precipitated calcium carbonate, whereas the last washings serve for dissolving the smelted compounds, thereby ensuring as complete a recovery of sodium constituent as possible.

As a result of the foregoing recovery or regenerating steps or any other recovery procedures with which I am familiar, the cooking liquor inevitably contains a substantial proportion of inactive chemicals, largely in the form of sodium carbonate and sodium sulphate. Thus, a typical causticized solution produced according to the regenerating process of my patent may contain 28% or even very much more inactive chemicals in the form of sodium sulphate and sodium carbonate, based on the total solids or chemicals present in the liquor. These inactive chemicals are of no benefit whatever in the cooking liquor, but as a matter of fact detract from the 15 pulping effectiveness of the liquor and impair the quality of the resulting pulp. The presence of sodium sulphate in the spent cooking liquor also tends to cause trouble in the pipe lines, pump, and evaporating system through which the liquor must be passed in order to arrive at the 20 concentration necessary for proper furnacing, as well as in the furnace itself, as will hereinafter appear in greater detail.

It is well for the purposes of the present invention to scrutinize carefully the conditions that prevail during a causticizing operation and that give rise to a causticized solution undesirably loaded, as hereinbefore described, with inactive chemicals. It is well known that the causticizing 25 reaction is one of the mass action type, depending as it does for its completion upon the solubility of the reaction products and the solubility of the reactants. The reactions taking place during causticization may be written as follows:—



The first reaction does not go to completion in mill practice for the reason that lime, a reactant, 30 is comparatively insoluble, being soluble to the extent of only 0.08 part in 100 parts of pure water at 100° C., whereas caustic soda, a reaction product, is infinitely soluble in water. The solubility of lime in water decreases progressively 35 as caustic soda is progressively added thereto, inasmuch as the hydroxyl ions furnished to the water by the caustic soda represses the solution and ionization of the lime. Accordingly, it will be clear that as the solution containing sodium 40 carbonate is progressively being causticized, the solubility of the lime effecting the causticization is progressively diminished until an equilibrium is reached when no further causticization of sodium carbonate will be effected even though 45 sodium carbonate remains present in substantial amount in the solution and there is a large excess of lime in the sphere of reaction. In the case of sodium sulphate, there is some reaction to form calcium sulphate, but inasmuch as the 50 calcium sulphate is more soluble than the lime, no precipitation of calcium sulphate can occur, though a small quantity of the more insoluble basic sulphate may be thrown out. It is for the foregoing reasons that in actual practice only 55 about 90% of the lime calculated to be theoretically necessary for the causticization of the sodium carbonate and the sodium sulphate present in the solution of smelted compounds is used. Such an amount of lime ensures all the precipitation 60 that can possibly take place under the conditions prevailing in mill practice so that if more lime is used, it is merely wasted. Under some conditions of concentration of the causticized solution, the caustic soda may throw out of solution some sodium carbonate and some sodium 65

hydrogen sulphide, but this is not a serious matter as the crystals of these compounds remaining in the causticizing tank are dissolved in the water used for washing the calcium carbonate sludge and are thus recovered.

In accordance with one phase of the present invention, causticization of the solution is performed as heretofore with lime, whereupon the work of causticization is completed through the use of barium sulphide and/or barium hydroxide 10 as the causticizing reagents. Such practice is illustrated as a flow sheet in Figure 1 of the accompanying drawings. In this connection, I wish to point out that both barium sulphide and barium hydroxide are quite soluble in water, far more 15 so than lime, and that barium sulphide is far less soluble than calcium sulphide. As previously stated, the causticized solution as it is delivered from the causticizing tanks contains caustic soda, sodium sulphide, and residual sodium 20 sulphate and sodium carbonate. To this solution is added the barium constituent in the form of barium sulphide and/or barium hydroxide theoretically necessary to convert substantially all of the residual sodium sulphate and sodium 25 carbonate into sodium sulphide and/or caustic soda, although it is preferable to use barium constituent slightly short of the theoretically calculated amount in order to avoid the presence of barium constituent in the cooking liquor and its 30 oxidation into insoluble barium sulphate which would contaminate the pulp. The barium sulphide and/or barium carbonate precipitate thus produced may be separated from the completely 35 causticized liquor and subjected to a reducing action in the presence of finely divided carbon or carbonaceous material in a kiln to reproduce the barium sulphide and/or barium oxide used in the second stage of causticization. The reactions which take place in the kiln are as follows: 40



When the precipitate is essentially barium carbonate or a mixture of barium sulphide and barium carbonate, it may be desirable to carry out the reducing action in the kiln in the presence of superheated steam so as to effect the following 50 reaction:



In those instances when the kiln is heated by producer gas, the foregoing reaction will take place anyway because the hydrogen content of the producer gas burns to form superheated steam as one of the products of combustion.

In effecting the last stage of causticization with barium sulphide, it should be noted that the products of such causticization consist of both caustic soda and sodium hydrogen sulphide, since barium sulphide hydrolyzes in water as follows:



Strictly speaking, neither barium hydrogen sulphide nor barium hydroxide are formed as compounds which can be separated from each other, both coexisting as barium hydroxy hydrogen sulphide having the formula  $\text{BaSHOH}$ , so that when I speak hereinafter, or in the appended claims, about barium hydrogen sulphide, I mean thereby to include barium hydroxy hydrogen sulphide. This latter compound does the causticizing work on the residual sodium sulphate and sodium carbonate present 70

in the solution according to the following equations:



The foregoing reactions tend to go to substantial completion by reason of the high solubility of the barium hydroxy hydrosulphide and the insoluble nature of the barium carbonate and the barium sulphate. In other words, the barium hydroxy hydrosulphide can complete the work of causticization initiated by the lime because it is far more soluble than the lime which, as previously explained, becomes more insoluble as the causticity of the solution increases until it is so insoluble that it can no longer effect causticization, at which time there is still a substantial amount of sodium sulphate and sodium carbonate left in the solution as well as residual undissolved lime. The question might be asked as to why calcium hydrosulphide, which is extremely soluble in water, cannot effect the same results as does the barium hydroxy hydrosulphide. The trouble with calcium hydrosulphide is, however, that upon being put into a solution of caustic soda, calcium hydroxide is immediately precipitated so that no better results are had than when lime is used to begin with. The causticizing action effected by barium hydroxide is, as in the case of barium hydroxy hydrosulphide, based upon the high solubility of this hydroxide and the insolubility of barium sulphate and barium carbonate. These reactions effected with barium hydroxide are well known to the chemist and need not be written herein.

There are many advantages inhering in a process practiced along the foregoing lines wherein lime is used to do all the causticizing work that it can and barium sulphide and/or barium hydroxide are then used to complete the work of causticization. Aside from the fact that the resulting causticized liquor is substantially free from inert chemicals like sodium sulphate and sodium carbonate that play no role whatever in the pulping of wood or other raw cellulosic material, it is possible to control with accuracy the composition of the causticized liquor and thereby to reproduce a given quality of pulp. Thus, if the sulphidity of the causticized solution is too great, this can be adjusted by adding sodium carbonate to the solution being causticized and/or by operating the furnace in which the smelting is effected under conditions to produce a greater amount of sodium carbonate. Indeed, the furnace may advantageously be run under oxidizing conditions substantially throughout to produce essentially only sodium carbonate in the smelt, inasmuch as it is possible through the use of barium sulphide in the last stages of causticization to form the desired amount of sodium sulphide in the causticized solution. This latter practice of operating the burning and smelting furnace without laying emphasis on the amount of sodium sulphide produced therein is of advantage in realizing maximum fuel value from the organic content being burned in a furnace of the type described in my aforementioned patent which is equipped with a boiler heated by the hot gaseous products of combustion produced in the furnace. Again, by running the furnace under oxidizing conditions, the reaction may more nearly approach an exothermic one throughout the furnace so that higher temperatures may be reached in the furnace and accordingly greater heating

efficiency realized with a given fuel value in the liquor. The higher temperatures realized in the furnace also means that the furnace has greater productive capacity. Moreover, the more nearly one approaches an oxidizing atmosphere throughout the furnace, the less is the wear and tear on the furnace walls. It is well known that fused sodium sulphide formed by maintaining a reducing atmosphere in the furnace is destructive of practically all the materials of construction that can be used in making the furnace walls and that the best that can be done in practice is to select wall materials known to be most resistant to the chemical action of the fused sodium sulphide. Aside from the chemical-corroding action of the fused sodium sulphide, its physical action is also highly destructive in that it tends to enter into the pores and interstices of the lining and to oxidize therein into sodium sulphate, which oxidation is accompanied by expansion and tendency to erupt the lining and slough off particles of lining material at its internal face. The sodium sulphide also tends to sublime and deposit on the boiler tubes and in the flue, in which localities it undergoes oxidation to form sodium sulphate which piles up so as to necessitate its frequent removal. The foregoing difficulties are minimized when the furnace is run with an oxidizing atmosphere substantially therethroughout, although some formation of sodium sulphide will inevitably ensue when sodium sulphate (salt cake) is added to the concentrated spent liquor as it is being delivered to the furnace.

The troubles encountered in the usual process are not confined to the furnacing operation, but extend, as previously indicated, to the cooking or pulping operation, as the cooking liquor contains substantial amounts of sodium sulphate and sodium carbonate which, on account of their inactivity, tend to interfere with the activity of the caustic soda and the sodium hydrosulphide. These inactive chemicals also cause serious trouble in other places in the system, as in the pipe lines, pumps, evaporators, explosion tanks, etc., for when the spent cooking liquor containing these chemicals reaches the last stages of concentration, these chemicals crystallize out and severely erode the metal parts with which they contact, particularly when the concentrated liquor containing the crystals is impinged forcibly as a spray against the metal parts, for instance, the metal parts of the last-stage evaporators, or is rapidly circulated, as it must be, past pipe and pump surfaces. The fact is that this problem of erosion gives rise to the need of using special hard steels as the material of construction of the pipe lines, pumps, gill flanges, evaporator heads, explosion tanks, and the various other parts of the system. The seriousness of the problem is increased when the ratio of inorganic solids to organic solids present in the spent liquor is increased as a result of handling a spent liquor which consists of a mixture of spent kraft cooking liquor and spent pulp-refining liquor, as will presently be described.

According to another phase of the present invention, I dispense with the addition of sodium sulphate to the concentrated spent liquor sent to the furnace to make up the losses of sodium and sulphur constituents in the cycle. By so doing, it is possible to operate the furnace in such a way as to realize an exothermic reaction therethroughout and the production of a smelt substantially devoid of sodium sulphide. To this end, instead of adding the make-up sodium sul-

phate to the concentrated spent liquor, I convert such sodium sulphate into sodium sulphide by effecting a metathetical reaction thereon in solution with barium sulphide. The barium sulphide used for effecting this metathetical reaction on the make-up sodium sulphate may be prepared, as hereinbefore described, by the reduction of barium sulphate in a kiln. The reaction products of the kiln contain not only barium sulphide, but also substantial amounts of residual barium sulphate and carbon. Nevertheless, the reaction products as a whole may be ground to a pulverulent condition, preferably in the presence of water to form a thick slurry, and the ground mass added to a solution of the make-up sodium sulphate to convert it into sodium sulphide. The sludge thereby formed containing barium sulphate and carbon is mixed with additional carbon and is returned to the kiln to reproduce barium sulphide. Should it be desired to produce substantially pure barium sulphate (*blanc fixé*) as a by-product, the kiln-reaction products are leached in water, the leach solution separated from the residual solids, and the solution then treated with elemental, finely divided copper so as to effect a reduction of the barium polysulphides present in the leach solution to the monosulphide stage, as disclosed in my application Serial No. 670,832, filed May 13, 1933. The desulphurization of the barium polysulphides present in the barium sulphide solution to the monosulphide stage is attended by a change of color of the solution from a canary or orange yellow to a water-white; and, when this water-white solution is used to effect the metathetical reaction on the solution of make-up sodium sulphate, the resulting barium sulphate precipitate is of such high whiteness and purity that it can be dehydrated and sold as *blanc fixé*. Such new barium sulphate and new finely divided carbon as is needed in the process may be added to the sludge separated from the leach water, and the mixture introduced into the kiln for reduction.

The sodium sulphide solution separated from the sludge may be added to the lime-causticized solution of the smelted compounds to produce a cooking liquor of the desired composition. In this connection, I wish to observe that when the make-up sodium sulphate is converted into sodium sulphide, as hereinbefore described, rather than being added to the concentrated spent liquor, it is possible to perform the causticization of the solution of smelted compounds with lime at such dilution as to reduce materially the amount of inactive chemicals, i. e., the sodium sulphate and sodium carbonate, in the lime-causticized solution. This reduces the amount of barium sulphide and/or barium hydroxide necessary to effect the second stage of causticization, which is performed as hereinbefore described. Despite the fact that causticization is thus carried out so as to produce a causticized liquor of lower than normal strength, nevertheless the concentration of solution desired for cooking, so far as concerns active chemicals, may be had by adding to such causticized solution the sodium sulphide solution produced from the make-up sodium sulphate at an appropriate higher concentration. By reason of the fact that a fresh cooking liquor thus prepared contains little inactive chemical, its concentration in terms of sodium constituent may be less than that of the usual cooking liquor and yet it may be a more effective pulping reagent than the ordinary fresh cooking liquor. For instance, in a typical kraft cooking liquor such as

has heretofore been used, 100 pounds of the liquor may contain 8 pounds of active chemical, assuming that the sodium sulphide as well as the caustic soda is active, and about 3.2 pounds or considerably more of sodium sulphate, sodium carbonate, and other inactive chemicals. According to the principles of my invention, by which such inactive chemicals are vastly reduced or substantially completely eliminated, it is possible to work with a cooking liquor containing less than 8 pounds of active chemicals per 100 pounds of cooking liquor and at the same time to realize a pulp of qualities superior to those of the usual kraft pulp. These improved qualities in the pulp are attributable to the fact that with the ordinary kraft cooking liquor, when the raw wood chips become saturated with cooking liquor, their pores and interstices are charged with inactive chemicals as well as with active ones so that the inactive chemicals occupy space in the chips which might otherwise be occupied by the active ones. In order to introduce into the chips sufficient active chemicals to effect a pulping action with the ordinary kraft cooking liquor, it is hence necessary to use a more concentrated liquor than is necessary when the pores and interstices of the chips are filled with a solution containing only active chemicals, as obtains when cooking liquors are prepared in accordance with my invention. Strictly speaking, the charging of the chips with active chemicals sufficient to ensure pulping or fiber liberation is not a space-displacement reaction but one which proceeds because of osmosis, as the raw wood chips are wet and the tendency is for chemicals in the cooking liquor to diffuse by osmotic pressure into the pores and interstices of the chips. The point is that when the cooking liquor contains only active chemicals, osmosis forces only active chemicals into the chips, whereas, when inactive chemicals as well as active ones are present in the cooking liquor, osmosis forces both kinds of chemicals into the chips so that it becomes necessary to provide a sufficiently higher concentration of active chemicals to increase the osmotic pressure tending to force active chemicals into the chips and thereby to arrive at an active chemical content in the chips adequate for the desired pulping action. Assuming that cooking liquors are prepared in accordance with my invention to contain as much active chemicals as the ordinary kraft cooking liquors, it is possible to effect a pulping action under given conditions of temperature and pressure in a shorter period of time than heretofore, wherefore, my invention makes possible an increased pulp reduction in a plant of a given digester capacity.

The principles of the present invention are also of great value when the production of kraft pulp is being carried on simultaneously with pulp-refining operations wherein alkaline liquors of the same general composition as kraft cooking liquors are used, as illustrated in the flow sheet designated as Figure 2 of the accompanying drawings. In refining preliberated wood pulp or the like with alkaline liquors, it is the practice to suspend the pulp in the alkaline liquors under time, temperature, and concentration of liquor conditions designed to effect the desired reaction upon and solution of the less resistant celluloses, including beta and gamma cellulose, lignin, resins, etc., from the pulp. As a result of such refining action, spent liquors are produced containing dissolved therein a comparatively small

amount of organic material. When such pulp-refining operations have been carried on in the same plant as the production of kraft pulp, it has been customary practice to use the spent refining liquor as part of the new cooking liquor in the kraft digesters. The refining liquor has been termed "spent" for the reason that it cannot be reused to advantage in refining pulp, but most of its alkali content being active, it can be used to good advantage as part of the kraft cooking liquor. The spent refining liquor is quite dilute by reason of the fact that the strong alkaline liquor of a composition similar to that used in kraft cooking is diluted when it is admixed with the aqueous suspension of the pulp to be refined thereby and is again diluted when the refined pulp is separated by washing from the spent refining liquor. The spent refining liquor contains sodium sulphate and sodium carbonate, because an alkaline liquor similar to the usual kraft cooking liquor has been used in the refining operation. It has been attempted to use the dilute spent refining liquor as part of the aqueous medium for dissolving the smelted compounds to be causticized, but this has occasioned trouble on account of the fact that the dissolved organic matter carried by the spent refining liquor inhibits to a great extent the settling of the calcium carbonate precipitated in the course of causticization. In other words, the dissolved organic matter coming from the spent refining liquor serves as a dispersing or stabilizing agent for the precipitated calcium carbonate, tending to keep it permanently in colloidal suspension. Accordingly, as already indicated, the best practice heretofore known was to circulate the spent refining liquor to the digesters so as to serve as one of the components of the fresh cooking liquor prepared therein. Because the spent refining liquor tends to throw out organic matter as its active chemical content is consumed during kraft cooking, the evaporating system becomes fouled by the deposition therein of such coagulated organic material as a fine powder; and the efficiency of the system is impaired as the organic matter accumulates therein along with crystallized solids more particularly in the last-stage evaporators, tending to coat the crystals and to keep the wash water used to clean the system periodically from getting at and dissolving the crystals.

I have found that it is possible to rid the dilute spent refining liquor substantially completely of its organic matter by adding thereto the ground kiln-reaction products as a concentrated slurry containing barium sulphide and/or barium hydroxide in amount greatly in excess of that theoretically necessary to convert the inactive chemicals present in the refining liquor, namely, the sodium sulphate and the sodium carbonate, into caustic soda and/or sodium hydrosulphide. Under these conditions, the dissolved organic matter is coagulated and the precipitated barium sulphate and barium carbonate entrains and carries down therewith the coagulated organic matter. The resulting causticized solution containing the residual large amount of barium sulphide and/or barium hydroxide may then be advantageously added to a sufficient amount of solution of the smelted compounds to react upon and consume all the residual barium sulphide and/or barium hydroxide in the causticization of the sodium carbonate and sodium sulphate present in the solution of smelted compounds, thereby producing a causticized solution containing no

barium constituent whatever. The sludge of barium sulphate and barium carbonate associated with organic matter is separated from the causticized refining liquor and is subjected to reducing action in a kiln, as hereinbefore described, to regenerate barium sulphide and/or barium oxide, the organic matter thus being consumed in the kiln rather than flowing through the system and functioning as a reducing agent in the reducing reaction effected in the kiln. The essential feature in such recovery procedure is the use of a large excess of the barium sulphide and/or barium hydroxide in concentrated condition in treating the dilute spent refining liquor, for I have found that when such refining liquor is added to the solution of smelted compounds and a treatment of the mixture is effected with barium sulphide and/or barium hydroxide, no coagulation of organic matter occurs and, moreover, there is a tendency to inhibit to a large extent the settling of the precipitated barium sulphate and barium carbonate. In other words, the barium sulphide and/or barium hydroxide function to coagulate the organic material only when they are present beyond a particular concentration, which particular concentration does not prevail when the refining liquor is admixed with a large volume of liquor containing the smelted compound before the addition of the barium sulphide and/or barium hydroxide. The causticized solution originating from a mixture of the refining liquor and the solution of smelted compounds and produced accordant with my invention may be used in preparing fresh refining liquor and fresh kraft cooking liquor, whereas the sediment of barium sulphate and barium carbonate is subjected to reducing action in a kiln, as previously described.

Once the principles of my invention have been put into practice in an already-operating kraft mill or in a kraft mill interrelated with a pulp-refining mill, it is possible to rid the system substantially completely of inert chemicals, namely, the sodium sulphate and/or sodium carbonate occurring in the liquor throughout the system. Of course, this will take place only after the liquor has gone through the complete cycle a number of times under the conditions of the present invention hereinbefore outlined. As the inert chemicals are eliminated from the system, the various troubles hereinbefore mentioned as being incident to the presence of such chemicals are done away with and such difficulties as arise from forcing the furnace to produce sodium sulphide are also avoided.

An important feature of the present invention is that the heated gases emanating from the kiln in which the barium sulphate and/or barium carbonate are being reduced can be advantageously utilized in decomposing the calcium carbonate resulting from the initial stage of causticization into lime. In this connection, I wish to point out that the reduction of barium sulphate and/or barium carbonate can be effected only at extremely high temperatures, whereas calcium carbonate can be decomposed into lime at much lower temperatures. The barium kiln is operated under conditions such that the gases emanating therefrom are at sufficiently high temperature and are of sufficient volume to effect a decomposition of substantially all the calcium carbonate put into the calcium kiln.

I have illustrated diagrammatically and conventionally in Figure 3 of the accompanying drawings two interconnected kilns running in

tandem, one kiln being for the barium and the other being for the calcium.

In Figure 3 of the accompanying drawings, the numeral 10 represents the barium kiln, which may be of the usual rotary type whose discharge end is journalled for rotation in a combined header and hopper 11 mounted on wheels 12 so as to be quickly removable from the discharge end of the kiln. The numeral 13 represents the calcium kiln, which may also be of the usual rotary type, whose discharge end is journalled for rotation in a sleeve or collar 14 having a hopper outlet 15. The intake end of the calcium kiln is journalled for rotation in the collar 14, being provided with an inwardly projecting annular flange 16 and being sufficiently spaced from the discharge end of the calcium kiln 13 to avoid commingling of the solid constituents of the two kilns. The intake end of the calcium kiln is journalled for rotation in a gas-receiver 17, being provided also with an inwardly projecting annular flange 18 for keeping the solid constituents in the kiln. Calcium constituent may be fed into the kiln 13 through a sluice 19 passing through the receiver 17 and discharging on the bottom of the kiln adjacent to the flange 18. Barium constituent may be fed into the kiln 10 through a sluice 20 passing through the upper wall of the collar 14 and discharging on the bottom of the kiln near the annular flange 16. Combustible gas, preferably producer gas, is delivered into the discharge end of the kiln 10 from a pipe 21 entering into the header 11. The air necessary for burning the gas may be introduced through a pipe 22 entering the side wall of the header. The pipes 21 and 22 may terminate at the same levels, as shown, whereat they may make a tight sliding fit with the corresponding supply pipes (not shown) so as to permit removal of the header from the discharge end of the kiln 10, as previously described. The removability of the header 11 from the discharge end of the kiln 10 is desirable for the reason that it makes possible the relining of both kilns and easy access to the interior of the barium kiln wherein sintering or partial clinkering of the solids may occur under the high temperatures prevailing therein so as to necessitate cleaning of the kiln or the removal of sintered obstructions therefrom. The gaseous products emanating from the intake end of the barium kiln, which pass through the calcium kiln, may require additional air for complete combustion so that a secondary air pipe 23 is shown entering into the upper wall of the collar 14 to deliver the volume of air requisite for this purpose. Both the hopper 15 and the hopper portion of the header 11 are preferably offset to one side so as to discharge the solid reaction products delivered thereto into suitable tanks stationed to one side and on a level below the kilns. The hopper 15 discharges into a comparatively large hopper-bottomed agitator tank 24 equipped with an inlet pipe 25 at its top, a power driven agitator 26, and a discharge pipe 27 at its bottom. The hopper portion of the header 11 discharges into a comparatively small hopper-bottomed agitator tank 28, also equipped with an inlet pipe 29 at its top, a power driven agitator 30, and a discharge pipe 31 at its bottom. Both kilns are arranged at a slight inclination to the horizontal, as is customary practice. The hot gaseous products of combustion coming from the intake end of the kiln 13 into the receiver 17 may be led through a flue 32 to a steam boiler for the recovery of as much of their heat content, as

possible, whereupon they may be used advantageously in drying the sludges going to the calcium and barium kilns, as their temperature is still sufficiently high for this purpose.

As previously stated, the initial stage of causticization of the solution of smelted compounds is productive of a sludge consisting essentially of calcium carbonate, but it is contaminated by small amounts of inert lime, sand, calcium silicate, etc. In order to avoid accumulation of impurities in the lime producible from the sludge, the sludge may be passed through a Dorr classifier which effects a separation of the impurities from the sludge so as to yield a substantially pure calcium carbonate suspension. The calcium carbonate suspension may then be thickened in any usual way, for instance, by settling and decantation or by a Dorr thickener, whereupon the thickened suspension may then be further reduced in its water content by passage through a filter, preferably a rotary filter of the Oliver type. The purified and thickened sludge of calcium carbonate, preferably after drying, as hereinbefore described, or after drying by any other hot flue gas, may then be passed through the sluice 19 into the kiln 13 for decomposition into lime. The sludge of barium carbonate, barium sulphate, and carbon resulting from the second stage of causticization may be thickened as on a rotary filter of the Oliver type, sufficient finely divided carbon or carbonaceous material added thereto to ensure the desired reduction to barium oxide and barium sulphide, and the mixture, preferably after drying as hereinbefore described, delivered through the sluice 20 into the kiln 10. The producer gas introduced into the kiln 10 for reducing the barium carbonate and barium sulphate to barium oxide and barium sulphide is burned with air to produce a maximum temperature in the kiln compatible with minimum sintering or clinkering of the solid reaction products, for instance, a temperature approaching about 2500° F. The producer gas is fed into the barium kiln in a volume sufficient to ensure the desired reduction in such kiln, which is accompanied by the liberation of carbon monoxide. The gases flowing into the calcium kiln from the barium kiln should be at sufficiently high temperature and should have a sufficiently large content of carbon monoxide and/or residual producer gas so that when they are burned in the calcium kiln with the secondary air furnished through the supply pipe 23, they will create a sufficiently high temperature and liberate sufficient heat to cause a substantially complete decomposition of the calcium carbonate in the calcium kiln. If sufficient air were added along with the producer gas in the barium kiln to consummate a substantially complete combustion of the producer gas and the carbon monoxide liberated in the barium kiln, an oxidizing atmosphere would exist at the discharge end of the barium kiln so as to preclude the desired reducing action thereat; and this difficulty would be aggravated by the lower temperature created thereat on account of the dilution with unnecessary comparatively cool air at this point. It is thus seen that the feature of adding secondary air to the incompletely burned gases entering into the calcium kiln is important from two standpoints, namely, that of ensuring the desired reducing action and temperature at the discharge end of the barium kiln and that of maintaining sufficient fuel value and/or a sufficiently high temperature in the gases flowing into the calcium kiln. It is further seen that the

barium kiln is maintained under the reducing atmosphere necessary therein, whereas the calcium kiln is maintained under an oxidizing atmosphere such as ensures a complete combustion of the 5 gases and a temperature conducive to the decomposition of the calcium carbonate into lime.

The hot lime delivered through the hopper 15 into the tank 24 is preferably admixed in such tank with the solution of smelted compounds 10 which may be supplied in suitable amount through the pipe 25, thereby performing the work of initial stage causticization in such tank. On the other hand, the tank 24 may be a comparatively small one and be supplied with only sufficient water 15 to convert the lime into a thick slurry capable of being pumped to storage tanks from which it may be delivered in the desired amount to a causticizing tank to which the solution of smelted compounds is sent. In either case, the commingling of the hot lime with water is accompanied 20 by the liberation of steam which rises through the hopper 15 into the kiln 13, thereby preventing carbon dioxide from reaching the tank 24 and carbonating the lime.

25 The mixture of barium oxide, barium sulphide, and residual barium carbonate, barium sulphate, carbon, and barium silicate, constituting the solid-reaction products of the kiln 10, are delivered into the comparatively small tank 28

30 which is supplied with an amount of water or preferably an amount of weak barium sulphide solution, presently to be described, to form a thick slurry or suspension which can be handled by a centrifugal pump and piped where desired.

35 As in the tank 24, there is an evolution of steam in the tank 28 as the hot reaction products commingle with the water sufficient to rise into the header 11 and thereby to prevent carbon dioxide from gaining access to the tank 28 and 40 carbonating the barium oxide or barium sulphide delivered thereinto. Should the steam liberated in either the tank 24 or the tank 28 be insufficient to preclude the entrance of carbon dioxide thereinto, additional outside steam

45 may be supplied thereinto for this purpose, as through a steam pipe 24a entering through the top of the tank 24 and as through a steam pipe 28a entering through the top of the tank 28. The thick slurry or suspension may be delivered

50 from the tank 28 to a ball mill, roller mill, or other pulverizing machine so as to reduce such clinkers as may be present in the slurry to fine particles whose soluble content, including barium oxide and barium carbonate may be leached out

55 by water. To this end, the slurry of fine particles discharged from the pulverizing machine may be used directly or be delivered to a dissolving tank whereto water in amount sufficient to ensure the solution of substantially all the

60 soluble compounds present in the slurry may be effected. The solution thus produced containing the insoluble residual barium carbonate, barium sulphate, carbon, and barium silicate in suspension therein, is separated from the

65 suspended solids and the slurry of solids is then run over a rotary filter of the Oliver type. The thickened slurry is washed on the same filter and the washings are preferably used, as hereinbefore described, for suspending the kiln-reaction products. The thickened slurry together with additional carbon and the slurry produced in the second stage of causticization, together with make-up barium sulphate, are fed through the sluice 20 into the barium kiln. The solution 70 of barium hydroxide and barium sulphide or the

pulverized slurry of reaction products from the barium kiln may be used for effecting the second stage of causticization, for coagulating organic matter from spent refining liquors, or for causticizing the make-up sodium sulphate, as has hereinbefore been described in detail. It will be appreciated that the tank 28 serves various functions, including that of permitting the white hot reaction products from the kiln 10 to be quenched therein, that of permitting the barium oxide to be hydrated therein, that of preventing carbonation of the barium oxide and barium sulphide, and that of a receiver in which the reaction products are converted to a form easily deliverable to other parts of the system.

While I have dealt with the application of the principles of the present invention to the production of kraft pulp and the regeneration of the spent chemical liquors arising therefrom either independently or correlated with the production of refined cellulose pulps and the regeneration of the spent chemical liquors resulting from the refining operation, nevertheless it is to be understood that they are applicable to the production of soda pulp and to the regeneration of the spent liquors arising therefrom, as in such case, too, one may advantageously resort to a two-stage causticization, the first stage of which involves the use of lime and is incomplete and the second stage of which involves the use 25 of barium hydroxide and goes to completion. Indeed, my invention may be extended to various processes of chemical pulp production and the regeneration of the spent chemical liquors resulting therefrom, so long as caustic soda is 30 one of the ingredients of the cooking liquor and causticization must be performed on sodium carbonate produced either by smelting the inorganic content of the spent cooking liquors or by reducing the spent cooking liquors to black 35 ash which is leached with water for the extraction of its sodium carbonate content. Indeed, my invention may be applied to any process wherein solution of sodium carbonate and/or sodium sulphate is to be causticized to completion. 40

I claim:—

1. A process which comprises first causticizing a solution of sodium carbonate and sodium sulphate with calcium hydroxide, and then treating the solution with barium hydrosulphide to convert residual carbonate and sulphate into hydrosulphide. 50

2. A process which comprises first causticizing a solution of sodium carbonate with calcium hydroxide, and then treating the solution with barium hydrosulphide to convert residual carbonate into hydrosulphide. 55

3. A process which comprises treating a solution containing dissolved organic matter with barium hydrosulphide, thereby coagulating the dissolved organic matter, said organic matter being that dissolved from cellulosic material and being present in sufficient concentration to be susceptible of the aforesaid coagulation. 60

4. A process which comprises treating a solution containing sodium carbonate and sodium sulphate wherein dissolved organic matter is present with barium hydrosulphide, thereby coagulating the dissolved organic matter and converting said sodium carbonate and sodium sulphate to sodium hydrosulphide, said organic matter being that dissolved from cellulosic material and being present in sufficient concentration to be susceptible of the aforesaid coagulation. 65

5. A process which comprises treating a solution containing sodium carbonate wherein dissolved organic matter is present with barium hydrosulphide, thereby coagulating the dissolved organic matter and converting said sodium carbonate to sodium hydrosulphide, said organic matter being that dissolved from cellulosic material and being present in sufficient concentration to be susceptible of the aforesaid coagulation. 5
10. 6. A process which comprises treating a solution containing sodium sulphate wherein dissolved organic matter is present with barium hydrosulphide, thereby coagulating the dissolved organic matter and converting said sodium sulphate to sodium hydrosulphide, said organic matter being that dissolved from cellulosic material and being present in sufficient concentration to be susceptible of the aforesaid coagulation. 10
15. 7. A process which comprises smelting the inorganic content of spent kraft cooking liquor to produce a smelt containing sodium carbonate and sodium sulphate, dissolving the smelt in water, causticizing the resulting solution with calcium hydroxide, and then treating the solution with barium hydrosulphide to convert residual carbonate and sulphate into hydrosulphide. 15
20. 8. A process which comprises smelting the inorganic content of spent sodium base cooking liquors to produce a smelt containing sodium carbonate, dissolving the smelt in water, causticizing the resulting solution with calcium hydroxide, and then treating the solution with barium hydrosulphide to convert residual carbonate into hydrosulphide. 20
25. 9. A process which comprises smelting the inorganic content of spent kraft cooking liquors to produce a smelt containing sodium carbonate and sodium sulphate, dissolving the smelt in water, causticizing the resulting solution with calcium hydroxide, and then reacting upon residual sodium carbonate and sodium sulphate in the resulting solution at least in part with barium hydrosulphide. 25
30. 10. A process which comprises smelting the inorganic content of spent sodium base cooking liquor to produce a smelt containing sodium carbonate, dissolving the smelt in water, causticizing the resulting solution with calcium hydroxide, and then reacting upon residual sodium carbonate in the resulting solution at least in part with barium hydrosulphide. 30
35. 11. A process which comprises smelting the inorganic content of spent kraft cooking liquor to produce a smelt containing sodium carbonate and sodium sulphate, dissolving the smelt in water, causticizing the resulting solution substantially as far as possible with calcium hydroxide, and then converting residual sodium carbonate and sodium sulphate in the resulting solution to sodium hydrosulphide by the addition of barium hydrosulphide thereto. 35
40. 12. A process which comprises smelting the inorganic content of spent sodium base cooking liquor to produce a smelt containing sodium carbonate, dissolving the smelt in water, causticizing the resulting solution substantially as far as possible with calcium hydroxide, and then converting residual sodium carbonate in the resulting solution to sodium hydrosulphide by the addition of barium hydrosulphide thereto. 40
45. 13. In interrelated pulping and pulp-refining operations involving the use of liquors containing caustic soda and sodium hydrosulphide as 45
50. 14. In the pulping of raw cellulosic material with liquor containing caustic soda and sodium hydrosulphide, those steps which comprise smelting the inorganic content of the spent pulping liquor to produce a smelt containing sodium carbonate, dissolving the smelt in water, causticizing the resulting solution substantially as far as possible with lime, and treating the lime-causticized solution with barium hydroxide and barium hydrosulphide to convert residual sodium carbonate present in the solution to caustic soda and sodium hydrosulphide, thereby reproducing a liquor for the pulping operation. 50
55. 15. In the pulping of raw cellulosic material with liquor containing caustic soda and sodium hydrosulphide, those steps which comprise smelting the inorganic content of the spent pulping liquor to produce a smelt containing sodium carbonate, dissolving the smelt in water, causticizing the resulting solution substantially as far as possible with lime, adding sodium sulphate thereto, and treating the solution with barium hydroxide and barium hydrosulphide to convert the sodium sulphate and residual sodium carbonate present in the solution to caustic soda and sodium hydrosulphide, thereby reproducing a liquor for the pulping operation. 55
60. 16. In a cyclic process, steps which comprise pulping raw cellulosic material in a solution containing caustic soda and sodium hydrosulphide, concentrating by evaporation the resulting spent pulping liquor, smelting the inorganic content of the concentrated liquor, dissolving the smelted compounds in water, causticizing the resulting solution with lime, and, by the action of barium hydroxide and barium hydrosulphide, converting residual uncausticized compounds present in the lime-causticized solution and tending to interfere with pulping, to crystallize out during the step of concentration, and to cause trouble during the step of smelting, into caustic soda and sodium hydrosulphide having far less such tendency before repeating the cycle. 60
65. 17. In a cyclic process, steps which comprise pulping raw cellulosic material in a solution containing caustic soda and sodium hydrosulphide, concentrating by evaporation the resulting spent pulping liquor, smelting the inorganic content of the concentrated liquor, dissolving the smelted compounds in water, and, by the action of both calcium hydroxide and barium hydrosulphide, converting practically all of such compounds into caustic soda and sodium hydrosulphide before repeating the cycle, thereby avoiding troubles in the pulping, concentrating, and smelting steps arising from the presence of residual uncausticized compounds in said solution of smelted com- 65
70. 75. 75

pounds when said solution is causticized only with calcium hydroxide.

18. In a cyclic process, steps which comprise pulping raw cellulosic material in a solution containing caustic soda and sodium hydrosulphide, concentrating by evaporation the resulting spent pulping liquor, smelting the inorganic content of the concentrated liquor, dissolving the smelted compounds in water, causticizing the resulting

solution with lime, and, by the action of barium hydrosulphide, converting residual uncausticized compounds present in the lime-causticized solution and tending to interfere with pulping, to crystallize out during the step of concentration, and to cause trouble during the step of smelting, into sodium hydrosulphide having far less such tendency before repeating the cycle.

HUGH K. MOORE.